

## 1

2,843,484

## ALKALIES FOR SINGLE POWDER PHOTOGRAPHIC DEVELOPERS

Ralph W. Baxendale, Rochester, N. Y., assignor to Eastman Kodak Company, Rochester, N. Y., a corporation of New Jersey

No Drawing. Application July 18, 1956  
Serial No. 598,526

9 Claims. (Cl. 96—66)

This invention relates to photographic developer compositions, the components of which are mutually compatible and can therefore be packaged for merchandising as a mixture in a hermetically sealed package. These photographic developer mixtures are commonly termed single powder photographic developers, and the present invention more particularly relates to single powder developers containing one or more alkali hydroxides which have been treated to lessen or to prevent their reactivity with components of the atmosphere as well as with other components of single-powder developers.

This invention also relates to methods of treating alkali hydroxides with one or more protectant compounds to lessen or to prevent interaction of the alkali hydroxide with the atmosphere, or with organic developing agents, as well as to the treated alkali products produced thereby.

In the past, photographic developer powders have been packaged so that the developing agents are separated from contact with the alkaline components to prevent interaction therebetween. More recently it has been found that some developer mixtures may be protected by the addition of certain protectants so that the developing agents may be mixed directly with other components of the developer and the resulting developer mixture can be packaged as a single powder developer.

Single powder developers may contain, for example, an organic developing agent such as monomethyl p-aminophenol sulfate, hydroquinone, p-aminophenol hydrochloride, p-aminophenol sulfate, pyrogallol, p-hydroxyphenyl glycine, catechol, diaminophenol hydrochloride, 1-phenyl 4-methyl-3-pyrazolidone, 1 phenyl 4,4-dimethyl-3-pyrazolidone and suitable mixtures thereof, stable alkaline buffer salts such as sodium carbonate monohydrate, sodium metaborate tetrahydrate ( $Na_2B_2O_4 \cdot 4H_2O$ ) and sodium tetraborate pentahydrate ( $Na_2B_4O_7 \cdot 5H_2O$ ); and protectants such as boric anhydride, metaboric acid, phthalic anhydride and sodium or potassium bisulfites and metabisulfites and may also contain the other well known ingredients normally present in a developer such as sodium sulfite and potassium bromide, the normal and known function of the alkali sulfite being that of preservative, lessening the oxidation in solution of the organic developing agent, while the known function of potassium bromide is that of a restrainer particularly inhibiting "fog" formation in the development of the silver image.

However, when employing sodium or potassium hydroxide in such protected single powder mixtures, the strongly hygroscopic nature of sodium hydroxide and the dampness of its surface has frequently been found to be the cause of discoloration even in the presence of the above-named protectants. This is particularly disadvantageous since it is often desirable to add a strong alkali such as sodium hydroxide to a developer powder to give a higher total alkalinity, or to add such strong alkali to single powder mixtures to overcome the acidity introduced by the protectants.

## 2

An object, therefore, of the present invention is to provide single powder developers containing an alkali hydroxide which has been treated so as not to react with atmospheric moisture or with the other components of the single powder developer.

Another object of this invention is to provide single powder developers containing sodium or potassium hydroxide from which developing solutions which are colorless, fully balanced and of a proper degree of activity can be prepared.

Another object of this invention is to provide a method of treating such alkali hydroxides to reduce their hygroscopic properties.

Yet another object is to provide a method of coating particles of alkali hydroxides with a nonhygroscopic coating which is also substantially inert in the presence of components of a single powder photographic developer.

Another object of this invention is to provide a non-caking sodium and potassium hydroxide having a coating thereon which is generated by a reaction between the selected alkali and an amide.

Another object of this invention is to provide single powder photographic developers containing sodium or potassium hydroxide which have been coated in accordance with the present invention with the reaction product of the selected alkali and an amide.

Other objects will appear hereinafter.

In accordance with a feature of the present invention these and other objects are attained by forming a coating on the selected alkali hydroxide by heating in the presence of an amide to a temperature until ammonia is produced as a byproduct. The ammonia being very volatile is easily expelled from the now coated alkali with which it does not react.

The preferred treatment involves employing an alkali hydroxide in particle form and an amide which on heating will produce ammonia as a byproduct. Suitable amides include urea, formamide, acetamide, propionamide, benzamide, phthalamide, oxamide. These form the corresponding alkali salts, the acetate, propionate, etc. Generally, weighed amounts of the reactants are employed. The reaction may be conducted in a rotary blender in a temperature range of 90 to 108° C. for approximately 60 minutes. The by-product, ammonia, is suitably removed from the reaction mixture. If desired, higher temperatures above 108° C., for example 120 to 140° C., may be employed to increase the rate of reaction.

The resulting product comprises an alkali hydroxide core having an adherent coating thereon and when this coated product is exposed to atmospheric conditions, it is found that the rate of moisture pick-up is very much slower than is the case with untreated alkali hydroxide. Such coated alkalies can be easily handled in the usual atmospheric conditions, whereas untreated alkalies become very damp after short exposure and eventually dissolve in the water which they absorb. The treated compounds can be packed in the soda portion of photographic developers without causing caking. When added to single powder photographic developer mixtures the treated compounds retard deterioration of the mixture and do not cause caking of the mixture.

The present invention will be further illustrated in the following examples:

## Example 1

A 1-kilogram lot of powdered sodium hydroxide was blended with 7.5 grams of urea and the mixture, in a rotary blender, was heated for 60 minutes in the temperature range of 90 to 108° C. The product was free from the dustiness and showed good handling properties. The thus coated sodium hydroxide was employed in a

single powder developer containing Elon (p-methylaminophenol sulfate) 2.5 grams, hydroquinone 5.0 grams, sodium sulfite 25.0 grams, borax 25.6 grams, potassium bromide 1.8 grams, and boric anhydride 1.3 grams and incubated at 120° F. for three weeks. No evidence of discoloration, which would indicate a reaction between the sodium hydroxide and one or more of the developing agents was noted.

*Example 2*

The coated sodium hydroxide of Example 1 was again mixed with 7.5 grams of urea and heated for 60 minutes in the temperature range of 90 to 108° C. This double treated product which exhibited no tendency to cake, was added to the same type of single powder developer as shown in Example 1, the amounts of the components being the same as in Example 1. No evidence of discoloration of the single powder developer was noted after 6 months incubation at 120° F.

*Example 3*

The double treated sodium hydroxide of Example 2 was again mixed with 7.5 grams of urea and heated for 60 minutes in the temperature range of 90 to 108° C. This triple treated product, which did not cake, was added to the same type of single powder developer, as mentioned in Examples 1 and 2 the amounts of the components being the same as in Example 1. The single powder mixture did not discolor after 6 months incubation at 120° F.

*Example 4*

Sufficient formamide to react with 1% of the sodium hydroxide was placed together with the sodium hydroxide in a flask. An exothermic reaction was found to proceed rapidly. This coated sodium hydroxide was added to the same type of single powder developer as described in Example 1, the amounts of the components being the same as in Example 1. The single powder mixture did not discolor after several months incubation at 120° F.

*Example 5*

Following the treatment with urea, as described in Example 1, the sodium hydroxide was then treated with dimethyl phthalate under the same conditions of mixing and temperature as in the case of treating with urea. Alkali hydroxides receiving one treatment with urea and two with dimethyl phthalate proved highly resistant to prolonged incubations when added to the developer powders as described above. The sodium hydroxide obtained was free flowing and relatively uniform in particle size.

*Example 6*

Examples 1 to 5 were repeated with potassium hydroxide and similar results were obtained.

*Example 7*

To illustrate further the use of the coated sodium hydroxide in photographic developer powder packing the following powder was prepared:

|                                 | Grams |
|---------------------------------|-------|
| Sodium sulfite, desiccated      | 22.5  |
| Sodium tetraborate pentahydrate | 25.8  |
| Potassium bromide               | 1.8   |
| Sodium hydroxide-urea treated   | 3.5   |

This mixture, which represents the salt portion of a photographic developer powder remained free flowing after storage of 6 weeks at 120° C. A similar powder in which untreated sodium hydroxide was used caked severely when stored under the same conditions.

*Example 8*

This example further illustrates the use of potassium hydroxide which has been treated with formamide in a

single powder mixture. The following single powder developer was prepared.

|                                            | Grams |
|--------------------------------------------|-------|
| Elon (p-methylaminophenol sulfate)         | 2.5   |
| Hydroquinone                               | 5.0   |
| Sodium sulfite (desiccated)                | 22.5  |
| Sodium tetraborate pentahydrate            | 26.3  |
| Potassium bromide                          | 1.8   |
| Phthalic anhydride                         | 1.2   |
| Potassium hydroxide treated with formamide | 0.7   |

When incubated at 120° C., this single powder mixture had no tendency to discolor or to deteriorate. A similar formula using untreated potassium hydroxide was unusable after the same incubation treatment.

Since the by-product in the reaction between the alkali hydroxide and the amide is ammonia which, at the temperature of the reaction, is expelled from the product, my present invention has a decided advantage over other processes for treating alkali hydroxides wherein water or an alcohol by-product remains with the product.

I claim:

1. The method of forming a non-hygroscopic coating on an alkali hydroxide which comprises heating the hydroxide with an amide selected from the group consisting of urea, formamide and phthalamide to form a thin coating of the reaction product of the hydroxide and the selected amide on the alkali hydroxide, and expelling the ammonia formed during the reaction.
2. The method of forming a non-hygroscopic coating on an alkali hydroxide selected from the group consisting of sodium and potassium hydroxide which comprises mixing the selected alkali hydroxide in comminuted form with an amide selected from the group consisting of urea, formamide and phthalamide and heating the mixture at a temperature to promote the formation of an integral non-hygroscopic coating of the reaction product of the hydroxide and the selected amide on the surface of the said alkali hydroxide and the expulsion of ammonia therefrom.
3. A stable single powder photographic developer composition which resists deterioration when heated to 120° F. containing an organic silver halide developer, a basic ingredient selected from the group consisting of alkali borates and sulfites and an alkali hydroxide selected from the group consisting of sodium and potassium hydroxide having a protective coating thereon of the reaction product of the selected alkali hydroxide and an amide selected from the group consisting of urea, formamide and phthalamide.
4. An alkali hydroxide having a coating thereon of the reaction product of the alkali hydroxide and an amide selected from the group consisting of urea, formamide and phthalamide.
5. Sodium hydroxide having a coating thereon of the reaction product of sodium hydroxide and an amide selected from the group consisting of urea, formamide and phthalamide.
6. Potassium hydroxide having a coating thereon of the reaction product of potassium hydroxide and an amide selected from the group consisting of urea, formamide and phthalamide.
7. Sodium hydroxide having a coating thereon of the reaction product of sodium hydroxide and urea.
8. Sodium hydroxide having a coating thereon of the reaction product of sodium hydroxide and formamide.
9. Sodium hydroxide having a coating thereon of the reaction product of sodium hydroxide and phthalamide.

References Cited in the file of this patent

UNITED STATES PATENTS

|           |         |               |
|-----------|---------|---------------|
| 150,509   | Babbitt | May 5, 1874   |
| 270,998   | Taylor  | Jan. 23, 1883 |
| 2,532,201 | Sprague | Nov. 28, 1950 |
| 2,639,221 | Henn    | May 19, 1953  |